

## UNITED STATES PATENT OFFICE

PRESCOTT H. WALKER AND SHERMAN S. KENYON, OF NIAGARA FALLS, NEW YORK,  
ASSIGNORS TO THE CARBORUNDUM COMPANY, OF NIAGARA FALLS, NEW YORK, A  
CORPORATION OF PENNSYLVANIA

## ABRASIVE OR REFRACtORY ARTICLES AND METHOD OF MAKING THE SAME

No Drawing. Application filed May 1, 1928. Serial No. 274,352.

This invention relates to an improved abrasive, refractory or other article made of a granular substance bonded with a suitable binder, more particularly a vitrified or ceramic binder, and to a method of producing them.

In the dressing of abrasive wheels, some of the trueing and dressing devices which have been used are of an abrasive nature and are

10 manufactured the same as the usual abrasive wheel or brick is manufactured. Consequently such trueing devices have been no harder and wear resistant than the hardest abrasive wheels. Therefore, the use of such 15 a device for trueing the grinding face of a wheel is only partially satisfactory because excessive wear makes it impossible to produce a grinding surface of the desired truth, shape or degree of sharpness.

20 Likewise, refractory articles, such as refractory bricks and shapes, and more particularly refractory articles composed of substances which are oxidized, decomposed or attacked by furnace gases in the presence 25 of which they are used, will have an increased life if they are less permeable, the life of refractories being more or less proportional to their permeability.

According to the present invention it is 30 proposed to increase the density or lessen the permeability of abrasive and refractory articles and, at the same time, modify or reinforce the binder or union between the binder and the granular materials in such manner 35 that the abrasive or refractory article is extremely wear resistant and has low permeability. An abrasive article made in accordance with our invention can be used with much greater efficiency as a trueing or dressing tool, or for other purposes where an extremely hard wear resistant abrasive article 40 is required. Not all methods of decreasing the permeability of an abrasive article have been found satisfactory because the density 45 of the composition can be decreased without necessarily increasing its wear resistant properties. For instance, it has heretofore been proposed to form an abrasive dressing tool with a large quantity of fine abrasive 50 grains in the mix so as to produce an article

of low permeability. Such an article, however, may not be highly wear resistant and in the case of an abrasive article is no more or but little more abrasive than those of the usual nature. Some such refractory articles 55 may not be highly wear resistant because of the possible weakening effect on the bond due to the oxidation of the fine particles.

According to our invention, it is proposed 60 to decrease the permeability of an article formed of a bonded granular substance by applying thereto some material which will impregnate the porous article and which will, itself, or some resultant product thereof, be interstitially deposited either by chemical 65 action or by addition or removal of heat, or combinations of such methods that the process will tend to fill the pores of the article or augment the binding properties of the bond and thus render the article less permeable 70 and more resistant.

An example of a satisfactory method of 75 decreasing permeability is the impregnation of a bonded abrasive article with a binder in liquid form, and the consequent setting of the binder. We have found that such materials as aluminum hydroxide and calcium hydroxide decrease the permeability satisfactorily when they are deposited in situ and the product subsequently burned. Other materials, such as alkali silicate solutions, or clay suspensions, or solutions of salts may be used to decrease the permeability.

80 As a specific example of the invention, a bonded abrasive wheel or stick used for dressing abrasive wheels is impregnated with a saturated solution of aluminum chloride and calcium chloride in the ratio of ten parts of aluminum chloride to one part of calcium chloride. The hydroxides of aluminum and calcium are then precipitated in the pores of the article by immersion of the article in ammonium hydroxide or by exposure of the article to ammonia vapors. The article is 85 then baked or burned to condition it.

90 It has been found that an abrasive wheel or stick used for dressing abrasive wheels treated in this manner will have its resistance to wear increased five or more times over that of the usual articles made for the purpose 95

and its permeability decreased greatly, sometimes as much as 100% or more. While the invention, as applied to abrasive articles, is particularly applicable to wheel trueing devices, it is also useful in the more common abrasive articles.

In the copending application of F. J. Tone, Serial Number 212,139, filed August 10, 1927, for a Low permeable refractory, and in the copending application of Benner and Easter, Serial No. 181,602, filed April 6, 1927, for improvement in Refractory articles and furnace lining made therefrom, certain methods are disclosed for increasing the density of refractories, including both aluminum oxide and silicon carbide refractories, but more particularly those refractories which are composed of substances which are oxidized, decomposed or attacked by the furnace gases to which they are exposed in use. It is pointed out in the said applications that the life of these refractories is more or less proportional to the permeability thereof.

The present invention may be used either alone or in conjunction with the processes of said copending applications to render a bonded granular article used as an abrasive much less permeable.

The article may be treated, as heretofore described in connection with abrasive articles. We prefer, however, in the treatment of refractories, particularly aluminum oxide refractories, to impregnate the bonded refractory article, either by painting or by dipping with a decomposable salt, such as a solution of aluminum sulphate. The impregnated article is then heated, either by a special heating operation or upon the first firing of the furnace in which the refractory is used, to a temperature approximating 800° C. The aluminum sulphate is decomposed and aluminum oxide is deposited in the pores of the brick in an extremely satisfactory manner.

The advantages of the invention reside in the fact that the permeability of the bonded granular article can be decreased greatly, sometimes 100% or more, and the article made highly wear resistant. Articles produced in accordance herewith have a permeability of less than 50 cubic centimeters. The invention can also be applied to an article composed of pulverant material and a binder and the advantages of the invention secured.

The permeability is measured according to any suitable method, that disclosed in said Benner and Easter application, Serial No. 181,602, preferably being employed. According to this method, air at a known pressure is applied to one face of the article to be tested and allowed to escape from the opposite face, the others being sealed by immersion in mercury. The air flow through the specimen is then measured by a meter in the air line ahead of the article. By multiplying the observed flow by the thickness of the

article, and dividing the product by the area and pressure, a unit of permeability is expressed in terms of air flow through a unit cube under unit pressure. As will be understood by those skilled in the art, the usual constants employed in determining the permeability factor is based on a thickness of one inch, an area of a square inch, giving a unit cube of one cubic inch and pressure is then exerted by one inch of water.

The invention is not limited to the particular materials nor the exact method described, as various changes and modifications may be made therein to secure the same advantages and such changes and modifications are within the contemplation of our invention.

We claim:

1. An abrasive article comprised of granular material and a binder, and having a filler in the pore space thereof substantially throughout the mass and having a permeability less than fifty cubic centimeters.

2. An article composed of granular abrasive particles and a binder, and having metallic oxide in the pores thereof distinct from the binder.

3. A ceramic article of low permeability comprising bonded granular particles and a non-oxidizable filling in the pores thereof throughout the mass, which filling is independent of and distinct from the medium which bonds the particles.

4. A bonded ceramic article of low permeability comprising a burned mass of granular particles and a binder, the pores substantially throughout the mass containing a heat resistant material which is distinct from the binder.

5. A method of producing ceramic articles of low permeability which consists in forming a bonded article of granular material and a binder, and then filling the pores of the article throughout the mass with an inorganic heat resistant substance distinct from the binder.

6. A method of producing ceramic articles of low permeability which consists in forming and maturing a bonded article of granular material and a binder, and then filling the pores substantially throughout the mass with a filler, and thereafter heating the article.

7. A method of producing ceramic articles of low permeability which consists in forming a bonded article of comminuted material and a binder, and then filling the pores substantially throughout the mass with a heat resistant oxide distinct from the binder.

8. The method of producing a ceramic article of low permeability which consists in forming a porous ceramic bonded article, filling the pores of said article with a fluid material and then decomposing the material

within the pores, and thereafter heating the article.

9. A method of producing a ceramic article of low permeability which consists in first forming and firing a porous ceramic article, then impregnating the pores of the article throughout substantially its entire mass with a fluid, and then treating the fluid material to effect a change therein to form a 10 filler within the pores of the article.

10. A method of producing a ceramic article of low permeability which consists in first forming and firing a porous ceramic article containing granular material and a bond, then impregnating the article with a 15 decomposable salt, then baking the article to effect a change in the decomposable material.

11. A method of producing a ceramic article of low permeability which consists in forming and maturing a bonded ceramic article, impregnating the pores of the article throughout substantially its entire mass with an aluminum salt, and then converting 25 the salt into a non-soluble material.

12. A method of producing a ceramic article of low permeability which consists in first forming a bonded ceramic article, impregnating the article with a salt in solution, 30 and then converting the salt into a non-soluble substance in situ within the pores of the article, and thereafter heating the article.

13. A method of producing a ceramic article of low permeability which consists in 35 impregnating the pores of the formed and matured bonded article throughout substantially its entire mass with a soluble material, then converting the soluble material in situ into a non-soluble filler.

14. A bonded and matured ceramic article 40 comprised of grains and a bond having a filler distinct from the bond in the pores thereof formed from a decomposable salt which has been subjected to the action of heat.

15. A bonded and matured ceramic article 45 comprised of grains and a bond having a filling material in the pores thereof comprised of a substance distinct from the bond precipitated in situ in the article.

16. The method of making a low permeable article comprised of granular material and a bond which comprises forming the article from the granular material and a bond, manufacturing the bond, thereafter impregnating the article with a soluble salt, precipitating an insoluble material in situ within the pores of the article from said salt and thereafter dehydrating the precipitate.

17. The method of reducing the permeability of a matured ceramic article containing granular material which comprises immersing the article in a solution containing aluminum and calcium salts, thereafter precipitating an insoluble filler from the salt

solution in situ in the pore spaces of the article, and thereafter heating the article to dehydrate the precipitated filler.

18. A hard abrasive article comprising bonded abrasive grains and a hard refractory material in the space between the bonded grains, said hard refractory material being formed in situ after the primary bonding whereby the density and hardness of the abrasive article are increased, the refractory material being distinct from the primary bonding agent. 70

19. The process of increasing the hardness and density of a bonded abrasive article which comprises immersing the article in a solution of a salt, precipitating a hydrate of said element by means of an ammonium compound in the pores of the article, and dehydrating the precipitate by the application of heat. 75

In testimony whereof we have hereunto set our hands.

PRESCOTT H. WALKER.  
SHERMAN S. KENYON.

85

90

95

100

105

110

115

120

125

130